

252/10544A1

Non-oxidizing acid  
+ abrasive

## United States Patent Office

3,248,235  
Patented Apr. 26, 1966

1

3,248,235

## ANTI-TARNISH COMPOSITION FOR COPPER-CONTAINING SURFACES

Donald M. Pryor and Louis F. Cason, both of St. Paul, Minn., assignors to Minnesota Mining and Manufacturing Company, St. Paul, Minn., a corporation of Delaware  
No Drawing. Filed Sept. 28, 1961, Ser. No. 141,292  
6 Claims. (Cl. 106—3)

This invention relates to an anti-tarnish composition for treating tarnished copper-containing surfaces and to a method for rendering such surfaces tarnish resistant.

Copper-containing surfaces, including copper alloys such as bronze, brass, etc., are notoriously susceptible to discoloration due to tarnishing of the copper. A great variety of copper cleaners have been suggested for the removal of tarnish deposits, e.g. copper oxides and sulfides. However, the problem of inhibiting the tarnishing of the cleaned copper-containing surface through the use of diverse polymers, lacquers, oils and waxes has not provided the prolonged tarnish resistance discussed or has had other serious drawbacks, such as discoloration of the protective coatings, difficulty in application, adverse effect on surface appearance, etc.

It is therefore an object of this invention to provide a clean, highly tarnish resistant copper-containing surface.

Still another object is to provide an anti-tarnish composition for application to copper-containing surfaces.

A further object is to provide a composition which simultaneously cleans copper-containing surfaces and renders such surfaces tarnish resistant for prolonged periods of time.

Yet another object is to provide a process for both cleaning and rendering copper-containing surfaces tarnish resistant.

Other objects and advantages will become apparent from the following description.

In accordance with this invention, a highly efficient composition for cleaning copper-containing surfaces and for rendering such surfaces tarnish resistant over an extended period of time comprises an aliphatic mercaptan of the formula  $C_nH_{2n+1}SH$  wherein  $n$  is from 12 to 25, preferably from 16 to 21, and at least one non-abrasive copper cleaning ingredient. If desired, other materials may be added to the composition, including suspending agents or surfactants, thickeners or viscosity improvers, abrasives, odorizers, solvent diluents and the like. The addition of other components as will suggest themselves to workers skilled in the art are considered to come within the contemplation of this invention.

In cleaning copper-containing surfaces various non-abrasive ingredients have been used to chemically remove the tarnish forming compounds. Conventional copper cleaners frequently contain mild organic acids, such as citric or sulfamic acid, together with sodium chloride, various surfactants and abrasives. After dissolution of the tarnish deposits by the non-abrasive copper cleaning ingredients, which are usually acidic, and dislodging imbedded tarnish by abrasive and/or surfactant action, if desired, the copper containing surfaces are extremely reactive in contact with the corroding environment. It is therefore preferable, for providing prolonged tarnish resistance, to accomplish the cleaning and the tarnish prevention simultaneously. Moreover, although abrasive containing mercaptan formulations effectively clean and condition the tarnished surface, the concentration or "loading" of abrasive required to remove the tarnish deposits tends to remove the protective mercaptan film as it is formed. The presence of non-abrasive copper cleaning ingredients permits the elimination of, or a reduction in,

2

the abrasive content of the formulation and provides significantly more effective tarnish resistance and a more efficient utilization of the mercaptan compound.

It has now been found that aliphatic mercaptans of the above formula provide a thin, colorless, non-oily protective layer on clean copper-containing surfaces, bonding to the copper through the thiol grouping, and that such mercaptans may be incorporated into copper cleaning formulations to provide a protective layer on the copper substrate as the tarnish is effectively removed by the cleaning ingredients. The bond between the copper and the mercaptans is unusually strong, resisting washing with dilute alkaline or acid solutions, and with detergent solutions. Of equal importance is the colorless, transparent protective layer of these mercaptan molecules, which does not adversely effect the luster of the copper-containing surface and which does not discolor or embrittle with aging. Moreover, although the film of mercaptan is virtually invisible to the naked eye, the presence of the protective layer may be detected by the hydrophobic or water repellent properties of the protected surface.

Both branched and straight chain aliphatic mercaptans may be employed, although the straight chain mercaptans are preferred. Mercaptans having less than twelve carbon atoms are not as desirable because of their somewhat greater volatility and greater difficulty in formulating with other desired cleaning ingredients. Mercaptans having more than twenty-five carbon atoms are not as desirable because they are higher melting solids and are more difficult to formulate. In general, these mercaptans have a mild odor which, if desired, may be masked with a suitable odorizer. They are non-toxic, particularly when considering the extremely minute quantities that are retained on the copper surface. Illustrative of the preferred mercaptans are n-hexadecane-1-thiol, n-dodecane-1-thiol, n-octadecane-1-thiol, n-benicosane-1-thio ( $C_{21}H_{42}SH$ ), etc.

Of the many non-abrasive copper cleaning ingredients which do not react with these mercaptans and which may be used in the anti-tarnish compositions of this invention the acidic cleaners are preferred because of their high efficiency. The various combinations of acidic ingredients suitable for cleaning copper-containing surfaces are well known. Generally, when using acidic cleaning ingredients in aqueous media, a pH of below about 2.5 is preferred. The combination of a weak acid, e.g., citric acid, sulfamic acid, etc., and an alkali metal halide, e.g., sodium chloride, potassium chloride, etc., is an effective non-abrasive tarnish remover. Hydrochloric acid also is also an effective non-abrasive copper cleaner. Since the anti-tarnish composition must be essentially non-oxidative, strong oxidizing acids, such as nitric acid, should not be used. Suitable acids having a pH between 1 and 5, which are water soluble, stable non-oxidizing acids which do not form water insoluble compounds with copper, as shown in U.S. Patent 2,628,199, are preferred.

The non-abrasive copper cleaners not only remove oxides from the tarnished copper surface but also permit the simultaneous formation of the continuous transparent film of the mercaptan compound. As mentioned earlier, when abrasives alone are employed in conjunction with the mercaptans compounds, the abrading effect tends to remove or disrupt the continuity of the protective film. Although abrasives may desirably be used in addition to the non-abrasive copper cleaners, particularly when heavy sulfide tarnish deposits are encountered, they constitute less than about 20 weight percent of the formulation and are preferably mild abrasives. Among the abrasive materials are finely divided silicas (including modified silicas), clays, diatomaceous earths, precipitated chalks, etc. In addition, small quantities of surfactant, particularly the nonionic variety, are usually employed. Viscosity

improvers and thickeners may also be incorporated into the formulation, and such thickeners as colloidal alumina (i.e., AlOOH) and guar gum are particularly effective in acidic media. The selection of thickener usually is dependent on the pH of the composition, since various thickeners are more stable at a given pH value than others. Among the thickeners are the natural gums (e.g., locust bean gum, guar gum), carboxymethyl cellulose, sodium alginate, hectorite, etc.

The cleaning and tarnish preventative compositions of this invention may be formulated as a liquid, as a solid stick or as a paste. For certain uses it may be desirable to impregnate fabrics with these anti-tarnish compositions to provide a convenient applicator cloth. It is also possible to dispense these compositions from pressurized containers, e.g., aerosols, etc.

Although the mercaptan, or mixture of mercaptans, can be incorporated in varying amounts into the compositions of this invention, depending partly on the physical nature of the formulation, it has been found that mercaptan concentration within the 0.5 to 25, preferably 0.5 to 10, weight percent range is particularly effective in formations containing a non-abrasive copper cleaner. Less than about 0.5 percent of mercaptan does not generally provide sufficient tarnish resistance.

In an aqueous liquid composition the most preferred formulations usually contain from about 1 to 15 weight percent of mercaptan, 0.01% to 25% of a weak organic acid, 0.01% to 25% of an alkali metal halide (e.g., alkali metal chlorides, etc.), 0.05% to 1% of a surfactant, 0 to 20% of an abrasive, sufficient water to emulsify the mercaptan, and sufficient acid stable thickeners to provide the desired viscosity.

The anti-tarnish composition may be applied to the copper-containing surface by spraying, dipping, roll coating, applicator cloth, etc. If an abrasive is included in the formulation, the copper surface is polished until the tarnish deposits are removed. When no abrasive is used, sufficient contact time is allowed to permit the copper cleaner to loosen and/or remove the tarnish, preferably followed by buffing or wiping to bring out the lustre of the copper surface. The removal of all tarnish is essential to obtain the continuous protective film required for extended protection of the surface. In all instances it is usually preferable to rinse the treated surface with water to remove any residual non-abrasive copper cleaner and abrasives. The following examples will illustrate the various preferred formulations, their use and effectiveness in preventing the tarnishing of copper-containing surfaces for prolonged periods.

#### Example I

Test panels of copper and brass were degreased with trichloroethylene and polished with a commercial copper cleaner containing a non-abrasive copper cleaner, i.e., citric acid and sodium chloride, to remove all traces of tarnish. Immediately after cleaning (a water rinse is preferable), the dry copper-containing surfaces were sprayed with a one percent solution of n-octadecane-1-thiol in petroleum ether and buffed with a soft cloth. The panels were then exposed to hydrogen sulfide at about 70% relative humidity along with cleaned uncoated control panels. A marked difference in tarnish rate was noticed, the deposits forming on the controls in less than 15 minutes and the coated panels remaining essentially tarnish free for several hours.

#### Example II

The procedure of Example I was repeated using n-heneicosane-1-thiol instead of n-octadecane-1-thiol. After exposure to the hydrogen sulfide atmosphere, the control panels (both copper and brass) tarnished in less than 15 minutes, whereas the treated panels were essentially tarnish free for several hours.

#### Example III

The following formulation was prepared, the percentages being by weight:

|                                                                 | Percent |
|-----------------------------------------------------------------|---------|
| 5 Water                                                         | 60      |
| Colloidal alumina (AlOOH)                                       | 3       |
| n-Octadecane-1-mercaptopan                                      | 10      |
| Citric acid                                                     | 8       |
| Sodium chloride                                                 | 8       |
| 10 Abrasive (50% diatomaceous earth and 50% of 240 mesh silica) | 10      |
| Nonionic surfactant                                             | 1       |

The colloidal alumina thickener was dissolved in water and the temperature raised to 80° C. After mixing the mercaptan and the nonionic surfactant and heating to 80° C., the mixture was added to the colloidal alumina solution with high speed mixing, forming a thick creamy emulsion. Once emulsification was complete, the citric acid and the abrasive were added with continued stirring until a homogeneous dispersion was obtained. Then upon adding the sodium chloride, immediate thickening to a smooth viscous paste occurred.

Copper panels were treated with the above formulation using a soft cloth, followed by water rinsing and air drying. Untreated copper panels which had been cleaned to remove tarnish were used as controls. After immersing both a treated and an untreated panel in a 1% aqueous solution of hydrogen sulfide, the untreated control was observed to tarnish after 5 seconds whereas tarnishing of the treated panel occurred only after about 2 hours. A similar comparative test using a salt bath (5% aqueous sodium chloride) resulted in tarnishing of the untreated control in 30 minutes and no visible tarnishing of the treated panel after two days. Still another comparative test was made by placing both treated and untreated panels in a high temperature (212° F.) oxidative (air) environment, resulting in tarnishing of the untreated control in 10 minutes and tarnishing of the treated panel only after 6 hours. In each of the foregoing comparative tests the time reported is the time required for visible signs of tarnish to appear.

#### Example IV

Results similar to those in Example III are obtained with the following formulation:

|                            | Percent |
|----------------------------|---------|
| Water                      | 76      |
| Hydrochloric acid          | 2.5     |
| Colloidal alumina          | 4       |
| 50 Abrasive                | 15      |
| n-Octadecane-1-mercaptopan | 2.4     |
| Nonionic surfactant        | 0.1     |

#### Example V

Results similar to those in Example III are obtained with the following formulation:

|                            | Percent |
|----------------------------|---------|
| Colloidal alumina          | 2.5     |
| n-Octadecane-1-mercaptopan | 2.4     |
| Citric acid                | 12      |
| Sodium chloride            | 12      |
| Diatomaceous earth         | 15      |
| Nonionic surfactant        | 1       |
| 65 Water                   | 55      |

#### Example VI

A composition for dip treatment of tarnished copper panels was prepared with the following ingredients:

|                            | Percent |
|----------------------------|---------|
| n-Octadecane-1-mercaptopan | 6       |
| Sodium chloride            | 15      |
| Citric acid                | 15      |
| Nonionic surfactant        | 1       |
| 75 Water                   | 63      |

Tarnished copper panels were immersed in the above formulation, agitation being used to stabilize the dispersion. Tarnish deposits were removed within a few seconds. The panels were then rinsed with water. Excellent resistance to tarnishing over an extended period of time was noted.

As used herein, "copper" is used interchangeably with "copper-containing" and includes, besides copper, such copper-containing alloys as brass, bronze, etc. having significant quantities of copper therein.

Various other embodiments and modifications will be apparent to those skilled in the art from the foregoing disclosure without departing from the spirit and scope of this invention.

We claim:

1. An aqueous anti-tarnish composition for copper which consists essentially of 0.01% to 25% of a weak organic acid, 0.01% to 25% of an alkali metal halide, 0.05% to 1% of a surfactant, 0 to 20% of abrasive, and 1 to 15% of a mercaptan of the formula



where  $n$  is an integer from 12 to 25, the pH of said composition being below about 2.5.

10

5 2. The aqueous anti-tarnish composition of claim 1 in

which said weak organic acid is citric acid and said alkali metal halide is an alkali metal chloride.

3. The anti-tarnish composition of claim 1 wherein the mercaptan is n-dodecane-1-thiol.

4. The anti-tarnish composition of claim 1 wherein the mercaptan is n-hexadecane-1-thiol.

5. The anti-tarnish composition of claim 1 wherein the mercaptan is n-octadecane-1-thiol.

6. The anti-tarnish composition of claim 1 wherein the mercaptan is n-heneicosane-1-thiol.

References Cited by the Examiner

UNITED STATES PATENTS

15 2,371,143 3/1945 Barnum ----- 148-6.24  
2,841,501 7/1958 Murphy ----- 148-6.24

OTHER REFERENCES

20 Bennett et al., "The Chemical Formulary," vol. I, pages 417-32, published by D. Van Nostrand Co., Inc., New York., 1933.

ALEXANDER H. BRODMERKEL, Primary Examiner.

JOSEPH REBOLD, MORRIS LIEBMAN, Examiners.

25